

Jan. 28, 1936.

K. GEPPERT

2,029,066

METHOD OF MEASURING THE HARDNESS OF ABRASIVE DISKS

Filed Oct. 31, 1934



Fig. 3.



Inventor:  
Karl Geppert  
per  
Blascheck, Danning & Seibold  
Att. 8

Patented Jan. 28, 1936

2,029,066

# UNITED STATES PATENT OFFICE

2,029,066

## METHOD OF MEASURING THE HARDNESS OF ABRASIVE DISKS

Karl Geppert, Schweinfurt-on-the-Main, Germany, assignor to Kugelfischer Erste Automatische Gussstahlkugelfabrik vorm. Friedrich Fischer, Schweinfurt-on-the-Main, Germany

Application October 31, 1934, Serial No. 750,901  
In Germany November 3, 1933

1 Claim. (Cl. 265—12)

Methods of measuring the hardness of abrasive disks, such as for example the scratching method, the impact method, the scraping method and the sand blast method are already known but they are all insufficiently reliable.

This invention enables the result of the test to be obtained with certainty to a very high degree of accuracy. A thin plate of perforatable material, such as for example, sheet metal, cardboard or pasteboard or the like, of any desired size is laid on the abrasive disk to be tested. A pointed conical impact pin, which is given one or a definite number of blows of uniform intensity perforates the plate and penetrates into the abrasive disk. The depth of penetration depends on the hardness of the abrasive disk. The resulting hole in the plate forms a qualitative record of the abrasive disk being tested in that the dimension of the diameter can be taken as the hardness number.

Fig. 1 shows a perspective view of the assembled parts for carrying out the invention;

Fig. 2 is a transverse sectional view of said assembled parts; and

Fig. 3 a plan view of a perforated plate used. In Figures 1 and 2 is shown an abrasive disk *a*, a thin plate *b* to be perforated and a punch or impact pin *c* with its conical point.

Both Figs. 1 and 2 show the plate *b* in position 5 on top of the abrasive disk *a* with the punch *c* after a blow has been applied thereon so that its point has penetrated the plate *b* and entered the disk *a*. A certain relation is thus established between the depth of penetration in the disk *a* 10 and the diameter of the hole produced in the plate *b*. The diameter of the resultant hole in the plate *c*, Fig. 3, will thus indicate the hardness of the abrasive material in disk *a*.

What I claim is:—

15 A method of measuring the hardness of abrasive disks or plates consisting in applying a sheet of perforatable material to the surface of said disk or plate, driving a conical impact pin through said sheet into said plate or disk by a standardized 20 driving force, and measuring the diameter of the perforation in the sheet.

KARL GEPPERT.